

Nov. 8, 1960

E. L. BAXTER ET AL

2,959,492

BACKING PAPER FOR ROLL PHOTOGRAPHIC FILM

Filed Feb. 13, 1959

**Fig. 1**



**Fig. 2**



**Fig. 3**



**Fig. 4**



**Ernest L. Baxter  
Martin Salo**

INVENTORS

*R. Frank Smith  
By Walter O. Hodden*  
ATTORNEYS

1

2,959,492

## BACKING PAPER FOR ROLL PHOTOGRAPHIC FILM

Ernest L. Baxter and Martin Salo, Rochester, N.Y., assignors to Eastman Kodak Company, Rochester, N.Y., a corporation of New Jersey

Filed Feb. 13, 1959, Ser. No. 793,177

4 Claims. (Cl. 117—14)

This invention relates to backing paper for roll photographic film, and more particularly relates to an improvement in the backing paper, described in Patent 2,751,309 of June 19, 1956, which has protective light-colored and opaques coatings thereon and is characterized by having an overall thickness appreciably less than conventional backing papers, and is superior in opaqueness to duplex backing paper.

As is well understood, a photographic roll film cartridge generally comprises a flanged spool upon which is wound a long strip of backing paper to which, before winding, has been attached on one side thereof a strip of light sensitive photographic film. The ends of the backing paper are positioned to extend beyond the ends of the film and constitute light protective leader and trailer strips for film which is interwound with the backing paper so that it separates adjacent convolutions of the film.

To assure opaqueness, backing paper conventionally employed for roll film consists of a duplex paper with one side being black and the other side being colored with a characteristic identifying color. The duplex paper may be made by means of a Fourdriner paper machine and a cylinder paper machine. The two sheets are brought together wet under the first press and thus form a composite sheet of duplex backing paper.

In a commonly available roll film cartridge, the film is attached to the black side of the duplex backing paper, the side of the backing paper opposite that contacting the film being differently colored and carrying various printed symbols such as the number of exposed areas, warning marks, and advertising matter over which is coated a protective layer intended to protect the sensitive emulsion from the paper and ink employed in printing when the film and paper are interwound in close contact. It has been the practice to depend entirely on the duplex paper to prevent transmission of light which would act on the film in the roll in loading and unloading the camera or through the camera window.

In the aforementioned Patent 2,751,309, there is described a new type of backing paper which, instead of a duplex paper, comprises a thinner, single sheet paper having unique chemical coatings thereon. This single sheet paper has a strength at least equal to the thinnest duplex papers now produced and an opacity equal to such duplex papers. The opacity is dependent primarily on the novel chemical coatings on the paper rather than the paper structure itself. This coated backing paper is also very flexible and the coatings withstand the winding incident to placing the backing paper and attached film on the spool.

As will be apparent from Patent 2,751,309, the black side of the backing paper comprises a layer either of carbon black in a vinylidene chloride-acrylonitrile copolymer or of carbon black in a styrene-butadiene copolymer.

Backing paper with a black layer made of carbon black in a styrene-butadiene copolymer is preferred, however, an unforeseen disadvantage was experienced with its use. Blocking of the styrene-butadiene to the zein coating on the opposite side occurs in the coating operation. Blocking also occurs between the styrene-butadiene coating and

2

the back surface of the roll film when spooled. In separating the backing paper and film in the processing operation, static discharges are produced on the film from this blocking action. Under conditions of high relative humidities and temperatures such as are encountered, for example, in the tropics, the back surface of the roll film becomes tacky with the result that it sticks to the surface of the backing paper with which it comes in contact. Under such extreme climatic conditions the sticking is occasionally so bad that chunks or areas of the black side are pulled off the paper. The photofinisher encountering roll film adhered to Duplex paper can, by prolonged washing and manipulation, wash off the black paper fibers and salvage some of the prints for the customer. When zein-carbon black, styrene-butadiene carbon black areas become cemented to the back surface of the film, it is extremely difficult for the photofinisher to remove these cemented portions and the customers' negatives, in most cases, are a complete loss.

20 We have found that the tacky back surface of the film under high humidity adheres very tightly to carbon black-zein layers as well as to numerous other types of materials.

An object, therefore, of the present invention is to provide an improved backing paper structure in which the advantages of the single sheet backing paper of Patent 2,751,309 are retained and the above-described static and sticking tendencies are eliminated.

Other objects will appear hereinafter.

In accordance with the present invention, these and other objects are attained by employing as the paper strip in the backing paper a single sheet, as contrasted to a duplex paper, which has been supercalendered to a thickness appreciably less than commonly employed duplex papers. By itself, this paper is so thin that it transmits sufficient actinic light to cause film exposure. This single paper is then coated on one side with a black opaque coating of carbon black in a styrene-butadiene binder which is then overcoated with carbon black in an ethyl cellulose binder. This carbon-ethyl cellulose layer will eliminate blocking of the backing paper and hence static difficulties occasioned thereby. The opposite side of the paper is coated with a plurality of lighter colored coatings. Printing may be placed on the lighter colored side of the backing paper and, if so printed, the printed side may be given a transparent protective overcoating to protect the film emulsion from the printing inks. The various coatings may be applied in proper sequence by a rotogravure process or by other suitable coating processes such as described hereinafter. The coatings may be suitably dried between applications.

50 The paper preferably employed as the base of the backing paper structure is a 14 pound per 1000 sq. ft. paper made of a purified fiber or of unpurified fiber such as unbleached natural color kraft paper which is conditioned to 4-12% moisture content and supercalendered to a thickness of 0.0025 to 0.0030 inch. The compositions of each of the black coatings and each of the light-colored coatings are further described hereinafter.

### BLACK COATINGS

The following two examples describe the composition of suitable black opaques coatings which are applied directly to one side of the paper:

#### Example I

|                                                                                              | Percent |
|----------------------------------------------------------------------------------------------|---------|
| Styrene-butadiene copolymer (50-70% styrene)<br>(48% solids in aqueous colloidal dispersion) | 21.6    |
| Carbon black                                                                                 | 14.8    |
| Sodium salt of partially desulfonated lignin sulfonic acid                                   | 0.75    |
| NaOH                                                                                         | 0.014   |
| Water                                                                                        | 62.8    |

## 3

## Example II

## Percent

|                                                                                              |      |
|----------------------------------------------------------------------------------------------|------|
| Styrene-butadiene copolymer (50-70% styrene)<br>(48% solids in aqueous colloidal dispersion) | 19.8 |
| Carbon black                                                                                 | 16.0 |
| Water                                                                                        | 63.3 |
| Sodium salt of partially desulfonated lignin sulfonic acid                                   | 0.80 |
| NaOH                                                                                         | 0.08 |

In preparing the black colored dispersions, the selected resin copolymers are added with stirring to a 30-40% aqueous carbon dispersion. The carbon dispersion is made by adding the carbon to water containing as a dispersing agent the sodium salt of the partially desulfonated lignin sulfonic acid and caustic soda is added to control the pH within the range of 10±1.

The black coating of Example II is preferred.

## BLACK OVERCOATING

## Example III

## Percent

|                 |      |
|-----------------|------|
| Ethyl cellulose | 5.0  |
| Carbon black    | 5.0  |
| Ethyl alcohol   | 90.0 |

This formulation is mixed by thorough stirring. A suitable ethyl cellulose is Dow Ethocel Type 10. It has a relatively low viscosity and a high solubility in ethanol. The resulting ethyl cellulose-carbon coating gives complete freedom from static and sticking.

## YELLOW COATINGS

The following three compositions may be employed for coating the light-colored side of the backing paper.

## Example IV

## Pounds

|                                  |     |
|----------------------------------|-----|
| Zein                             | 20  |
| Medium chrome yellow             | 10  |
| Light orange (chrome)            | 5   |
| Titanium dioxide                 | 15  |
| Isopropyl alcohol                | 64  |
| Water                            | 16  |
| Staybelite (hydrogenated rosin)* | 1.2 |

\* A pale, medium hard, thermoplastic resin made from hydrogenated wood rosin; acid number 162; softening point 76° C.; density 1.045 at 20° C.

## Example V

## Percent

|                                                                                       |       |
|---------------------------------------------------------------------------------------|-------|
| Styrene-butadiene copolymer (50 to 70% styrene)<br>(48% solids in aqueous dispersion) | 9.4   |
| Medium chrome yellow                                                                  | 37.5  |
| Titanium dioxide                                                                      | 9.3   |
| Lecithin                                                                              | .94   |
| Triton X-100 (alkylated aryl polyether alcohol)                                       | .47   |
| Carboxy methyl cellulose                                                              | .37   |
| NaOH                                                                                  | .05   |
| Water                                                                                 | 42.00 |

## Example VI

## Percent

|                                                                        |      |
|------------------------------------------------------------------------|------|
| Vinylidene chloride-acrylonitrile copolymer latex<br>(51.5-53% solids) | 19.2 |
| Medium chrome yellow                                                   | 12.6 |
| Titanium dioxide                                                       | 12.6 |
| Tamol (sodium salt of condensed sulfonic acid)                         | 1.3  |
| Sodium hydroxide                                                       | 0.4  |
| Water                                                                  | 53.9 |

In these formulas the titanium dioxide pigment is finely divided; medium chrome yellow is a finely divided metal chromate pigment; light orange is a finely divided metal chromate pigment. Zein is employed as the binder in the yellow coating of Example IV and the protective overcoating, since it will not fog or desensitize the photographic emulsion of the film.

## 4

A suitable rotogravure process for applying these coatings to the paper base of the backing paper is described in U.S. Patent 2,218,249 of October 15, 1940. The various applications are made continuously and each 5 coating is dried before the next is applied. The coating is applied to the paper by the intaglio roll which is rotatably mounted in a pan containing the coating solution. The surface of the intaglio roll is embossed, providing a plurality of very minute cups which carry the 10 solution, the excess solution being removed from the intaglio roll by a doctor blade. The solution in these various cups is then transferred or applied uniformly to the strip by pressing the strip firmly against the cups by means of a rubber pressure roll over which the strip 15 is fed. Each of these deposits, after being placed on the paper, is merged into a continuous layer by means of a smoothing bar to provide a uniform coating over the entire paper surface. Each coating is preferably dried in heated air having a relative humidity of 6% at 170° 20 F. before applying a second coating.

The various coatings described herein may also be applied to our backing paper base by the roll and air knife method generally described in Patent 1,980,923 of November 13, 1934. The selected black coating is applied first to one side of the single sheet backing paper 25 and spread by the air knife. This black coating is dried at 180-200° F. by being passed through a heated drying chamber. In some instances a plurality of black coatings may be spread onto the black side of the backing paper 30 by alternate coating and drying steps.

Suitable ink compositions for printing indicia by rotogravure processes on the backing paper are disclosed in Patent Re. 21,268 of November 21, 1939. These inks comprise suitable coloring materials in a prolamine binder 35 such as zein. Other suitable printing inks for such backing papers are disclosed in Patent 2,262,987 of November 18, 1941.

The invention will be further understood by reference to the drawings in which Figs. 1 to 3 represent a greatly 40 enlarged cross-section of backing paper made in accordance with various forms of the present invention and Fig. 4 shows the novel backing paper of Fig. 1 and photographic film wound on the roll with the film and backing paper separated at one end for purpose of illustrating 45 their relative positions in the roll.

Referring to Fig. 1, a cross-section of a strip of bleached kraft paper is shown at 10 having on the lower surface thereof a coating 11 of a layer of carbon black in styrene-butadiene copolymer coated from the composition of Example I. Layer 11 is overcoated with a layer 50 12 of carbon black in ethyl cellulose which is coated thereon from the composition of Example III. On upper surface of the paper 10, there is the yellow coating 13 comprising chrome orange and yellow pigments as well as titanium dioxide pigments in a zein binder. This was coated from the composition described in Example IV, supra. The printed indicia is shown at 14 overcoated with a transparent protective zein coating 15. Such a transparent zein protective coating is described in Patent 60 2,262,987 of November 18, 1941 and is also employed in layers 25 and 35 of Figs. 2 and 3.

Referring to Fig. 2, a cross-section of a strip of bleached kraft paper is shown at 20 having on its lower surface a coating 21 of a layer of carbon black in the styrene-butadiene copolymer coated from the composition of Example II. Layer 21 is overcoated with a layer 65 22 of carbon black in ethyl cellulose which is coated thereon from the composition of Example III. On the opposite surface of the paper 20 there is a yellow coating 23 comprising chrome yellow and titanium dioxide in a styrene-butadiene binder. This was coated from the composition described in Example V. The printed indicia is shown at 24 overcoated with a transparent zein coating 70 25.

Referring to Fig. 3, a cross-section of a strip of

bleached kraft paper is shown at 30 having on its lower surface a coating 31 of a layer of carbon black in the styrene-butadiene copolymer coated from the composition of Example II. Layer 31 is overcoated with a layer 32 of carbon black in ethyl cellulose which is coated thereon from the composition of Example III. On the upper surface of the paper 30 there is a yellow coating 33 comprising medium chrome yellow and titanium dioxide in a vinylidene chloride-acrylonitrile copolymer. This was coated from the composition described in Example VI. The printed indicia is shown at 34 overcoated with a transparent zein coating 35.

The backing paper structure described in connection with Fig. 1 is the preferred form of the present invention. However, the backing paper structure shown in any of the Figs. 1 to 3 gives a product that fulfills all the advantages herein, at an economical cost and results in a non-blocking, non-dust producing backing paper when stored under conditions of high humidities and temperatures or when wound through a camera.

Referring to Fig. 4, a film cartridge 40 is shown partly open in which the backing paper of the present invention is employed. This drawing shows the relation of the backing paper surfaces 15 and 12 of Fig. 1 in respect to film 43 when assembled on the spool 40. The emulsion side of the film is shown at 41 and the base side at 42.

While the preferred coating compositions are described above, satisfactory backing papers may be made by employing the various coating materials in the following ranges:

Preferred range  
of total composition  
percent

Compositions:

|                                                                            |          |
|----------------------------------------------------------------------------|----------|
| Vinylidene chloride-acrylonitrile copolymer of styrene-butadiene copolymer | 5 to 25  |
| Black pigment                                                              | 1 to 20  |
| White pigment                                                              | 15 to 45 |
| Yellow pigment                                                             | 15 to 45 |
| Water                                                                      | 50 to 70 |

Other useful pigments are, for example, Hansa Yellow, Fast Pigment Yellow and any carbon black of suitable dispersion.

Other pigments which are inert to photographic emulsions may be employed. In fact, any choice of pigments of suitable size for this invention is limited only by the requirement that they be without detrimental effect on the photographic film.

THICKNESS OF COATING

Black coating composition is applied in two coatings to give a total of 12 lbs. of solution per 1000 sq. foot for satisfactory opacity.

Light pigment composition is applied in the amount of 5 lbs. per 1000 sq. foot to give satisfactory uniformity of color.

The ethyl cellulose-carbon black coating is applied in .18 lb. per 1000 sq. foot.

Any other type of paper may be employed if it has good strength at least comparable to the present duplex paper. A rag paper, for example, is suitable but, of course, more expensive than kraft paper.

COMPARISON OF DUPLEX AND KRAFT TEAR STRENGTH

|                                                    | Elmendorf Tear |                 | Schopper Folds |        |
|----------------------------------------------------|----------------|-----------------|----------------|--------|
|                                                    | along,<br>gms. | across,<br>gms. | along          | across |
| Typical Duplex Paper                               | 70             | 84              | 410            | 28     |
| Kraft Paper (as employed in the present invention) | 76             | 93              | 295            | 115    |

Preferably the average tear strength of a suitable paper should be at least 50 gms. as determined by the Elmendorf tear test. This tear test is described in Paper Trade Journal for June 18, 1942 as Tappi Standard T414M40.

5 While, as indicated above, kraft paper is particularly suited for employment in my invention, certain other types of paper could be employed instead, such as unbleached sulfate paper colored with a suitable dye such as Stilbene yellow in which a small amount of filler such as  $TiO_2$  is added to give body and density or opacity to the paper.

These papers comprising the base of the backing paper are of a weight that can be supercalendered to a thinness that the paper itself plus the coatings thereon does not exceed an average maximum thickness of 0.0040 inch. A 15-pound per M sq. ft. paper has been found satisfactory.

The opacity of roll film backing paper is tested in the following manner.

20 A sheet of the backing paper under test is placed over a sheet of highly sensitive film, such as Super XX Pan-chromatic film with the black side of the backing paper in contact with the back of the film, duplicating its position on roll film. An orange-red filter of the type employed in camera back windows is placed over the opposite side of the backing paper and the assembly is placed in a printing frame. The test material is exposed to a light intensity of 5000 foot candles for ten minutes. The film is then processed in the usual way and examined for the presence of specks of developed silver. A satisfactory backing paper should show no visible silver image.

The improvement in employing the resinous coatings of the present invention as respects flexibility is shown in the following table:

|                                                              | Taber<br>Stiffness <sup>1</sup> | Clark<br>Stiffness <sup>2</sup><br>dbl. sample |
|--------------------------------------------------------------|---------------------------------|------------------------------------------------|
| 40 Butadiene-Styrene, black-Zein, yellow pigmented           | 1.95                            | 55                                             |
| Butadiene-Styrene, black-Butadiene-Styrene, yellow pigmented | 1.85                            | 38                                             |
| Zein Yellow on Black Paper                                   | 4.30                            | 89                                             |
| Red and Black Duplex Paper                                   | 5.10                            | 134                                            |
| Green and Black Duplex Paper                                 | 4.85                            | 133                                            |

(The higher the number the stiffer the paper.)

<sup>1</sup> Tappi Tentative Method T-451.

<sup>2</sup> Tappi Instrumentation Studies XIV.

50 We have found that our improved backing paper has many advantageous features not possessed by duplex papers which it may replace. The strength and other physical properties of the paper employed as the base of the backing paper is at least equal to the strength of the thinner duplex papers now available to the trade.

55 The overall thickness can be made as low as 0.0032, up to 0.0045 inch thus permitting extra exposures to be added to present rolls of film without increasing the diameter beyond that of films now in use. The opacity, even though the overall thickness is less than backing papers now available in the trade, is better than such

60 backing papers. The backing paper made in accordance with our invention requires the least amount of coating materials, both black and colored, of any of the methods described or known in the trade. The uniformly light-

65 colored side gives maximum contrast with the legends printed thereon. Also less clock springing of freshly rolled film is experienced with this paper than with the thicker duplex paper. The additional coating of the ethyl cellulose-carbon black on the black side of the

70 backing paper solves the difficulty of blocking between adjacent convolutions of the roll and eliminates static discharges. These advantages plus the advantage of applying the coatings by rotogravure and air knife methods, which are fast, accurate and efficient, emphasize the importance of my present invention in this art.

We claim:

1. In photographic backing paper having an overall thickness less than 0.0045 inch consisting of a single sheet of thin kraft paper which is of a thinness which will permit passage of substantial amounts of actinic light, having on one side a light colored pigmented coating consisting essentially of a yellow pigment in a binder selected from the class consisting of vinylidene chloride-acrylonitrile copolymer, styrene-butadiene copolymer and zein, printed indicia on said lighter colored coating, a clear zein protective coating thereover, and on the opposite side an opaque coating consisting of carbon black in a binder of styrene-butadiene copolymer, the improvement which consists in a protective coating over said opaque coating of carbon black in ethyl cellulose.

2. In photographic backing paper having an overall thickness less than 0.0045 inch consisting of a single sheet of thin kraft paper which is of a thinness which will permit passage of substantial amounts of actinic light, having on one side a light colored pigmented coating consisting essentially of a yellow pigment in a binder of vinylidene chloride-acrylonitrile copolymer, printed indicia on said lighter colored coating, a clear zein protective coating thereover, and on the opposite side an opaque coating consisting of carbon black in a binder of styrene-butadiene copolymer, the improvement which consists in a protective coating over said opaque coating of carbon black in ethyl cellulose.

3. In photographic backing paper having an overall thickness less than 0.0045 inch consisting of a single sheet of thin kraft paper which is of a thinness which will permit passage of substantial amounts of actinic light, hav-

ing on one side a light colored pigmented coating consisting essentially of a yellow pigment in a binder of styrene-butadiene copolymer, printed indicia on said lighter colored coating, a clear zein protective coating thereover, and on the opposite side an opaque coating consisting of carbon black in a binder of styrene-butadiene copolymer, the improvement which consists in a protective coating over said opaque coating of carbon black in ethyl cellulose.

10 5 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

## References Cited in the file of this patent

## UNITED STATES PATENTS

|           |               |               |
|-----------|---------------|---------------|
| 1,300,056 | Tyrrell       | Apr. 8, 1919  |
| 1,915,391 | Stoops        | June 27, 1933 |
| 2,227,843 | Quenelle      | Jan. 7, 1941  |
| 2,331,715 | Nadeau et al. | Oct. 12, 1943 |
| 2,340,971 | Manley et al. | Feb. 8, 1944  |
| 2,751,309 | Baxter        | June 19, 1956 |